

## UNITED STATES PATENT OFFICE

2,603,603

AGENTS AND MINERAL OIL LUBRICANT  
COMPOSITIONS CONTAINING THE SAME

Herschel G. Smith, Wallingford, and Troy L. Cantrell, Lansdowne, Pa., assignors to Gulf Oil Corporation, Pittsburgh, Pa., a corporation of Pennsylvania

No Drawing. Application December 27, 1946,  
Serial No. 718,902

12 Claims. (Cl. 252—46.6)

1

This invention relates to improvement agents and mineral oil lubricant compositions containing the same and, more particularly, it is concerned with improvement agents which confer improved antioxidant, corrosion-inhibiting and pressure-carrying properties on mineral oil lubricants.

It is recognized in the art that mineral oil lubricants are readily oxidized under service conditions thereby reducing the service life of internal combustion engines and steam turbines. A concomitant effect is corrosion of bearing surfaces. These problems become particularly acute when a highly refined paraffinic base mineral oil is employed as the lubricant.

In the lubrication of internal combustion engines of all types, particularly when severe operating conditions are encountered, mineral lubricating oils frequently prove unsatisfactory because they tend to deposit varnish, gum and sludge on the engine surfaces, such as the cylinder walls, piston and rings, and also to induce corrosion of bearing materials thereby causing failure of the engine. These problems have become increasingly serious because of the trend toward higher efficiency or higher power output per unit weight of engine, which results in conditions tending to accelerate the deteriorating influences on the mineral oil lubricant. The formation of so-called varnishes and sludges on engine surfaces is a result of oxidation effects on the lubricating oils. The presence of gums, varnishes and sludges is detrimental for many reasons. These substances tend to increase ring sticking and accelerate the formation of further deposits on piston surfaces and in fixed parts of the combustion chamber. The sludges formed in the crank case of the engine increase the rate of corrosion of bearing surfaces, especially of bearing alloys of the types now in use.

In steam turbines, the corrosion problem is particularly acute because of the presence of water in the mineral oil lubricant, and in addition to bearing corrosion, rusting may also be encountered.

It is an object of this invention, therefore, to prepare an improvement agent which will obviate the oxidation and corrosion difficulties encountered in the use of mineral oil lubricants.

It is a further object of this invention to provide improved mineral oil lubricant compositions which are stable in storage and use and in which oxidation and corrosion effects are materially inhibited.

It is also an object of this invention to provide mineral oil lubricant compositions which have excellent pressure-carrying properties.

These and other objects are achieved by the

2

present invention wherein an improvement agent for mineral oil lubricants is prepared by heating an essentially paraffinic base lubricating oil with anhydrous aluminum chloride, removing aluminum chloride from the reaction product, and reacting said product with phosphorus pentasulfide at an elevated temperature to incorporate phosphorus and sulfur therein.

We have found that the reaction product of phosphorus pentasulfide with an essentially paraffinic base lubricating oil which has been treated with aluminum chloride produces an improvement agent for mineral oil lubricant compositions which is remarkably effective in inhibiting oxidation and corrosion and which, in addition, confers excellent pressure-carrying properties on mineral oil lubricants. Such improvement agents, as well as the mineral oil lubricant compositions containing them are believed to be novel and are considered parts of our invention.

In the production of our new improvement agents, we have found that the treatment of an essentially paraffinic base lubricating oil stock with anhydrous aluminum chloride prior to reacting the product with phosphorus pentasulfide is critical. If the treatment with aluminum chloride is omitted and a paraffinic base lubricating oil is reacted with phosphorus pentasulfide, there is obtained a black, sludge-like product which is poorly soluble in mineral lubricating oils and which imparts such a degree of color to mineral oil lubricant compositions as to render them unmarketable. The same disadvantageous effects are observed when a hydrocarbon other than an essentially paraffinic base lubricating oil is used as the initial material. On the other hand, when anhydrous aluminum chloride is used to treat an essentially paraffinic base lubricating oil prior to its reaction with phosphorus pentasulfide, there is obtained on subsequent reaction a clear, light-colored, readily soluble product which may be incorporated into mineral lubricating oils without substantially affecting the color thereof, and which, at the same time, confers improved pressure-carrying, antioxidant and corrosion-inhibiting properties.

The reasons for the remarkable effects of the aluminum chloride treatment are not fully understood. It is known in the art that the treatment of hydrocarbon oils with anhydrous aluminum chloride tends to cause isomerization and an effective decrease in the unsaturation of such hydrocarbon oils. It is also known that aluminum chloride treatment of higher boiling hydrocarbons under drastic conditions converts such hydrocarbons into lower boiling products. The extent of any or all of these reactions in

our process is unknown except that substantial conversion of higher boiling hydrocarbons to lower boiling products is avoided. We do not desire to be bound, therefore, by any theory of the action of anhydrous aluminum chloride on the paraffinic base lubricating oil reactant material. However, the aluminum chloride treatment is essential for the practice of our invention, since without such treatment the advantageous results of our invention are not obtained.

The essentially paraffinic base lubricating oil used as a starting material may be derived from any paraffinic crude, such as a Pennsylvania, Mid-continent or other paraffinic base crude. The lubricating oil is manufactured from such crude in accordance with conventional methods and may be refined in accordance with methods known in the art. Treatment with aluminum chloride in accordance with our invention is accomplished by heating the essentially paraffinic base lubricating oil with from 1 to 20 per cent of anhydrous aluminum chloride at a temperature of from 150° to 300° F. while vigorously agitating. The time of treatment may vary in accordance with the amount of aluminum chloride used and the temperature of treatment, longer times being required with less aluminum chloride and lower temperatures. In general, however, the treatment will be completed after 4 or 5 hours. In any event, treatment is continued until a product is obtained which, when freed of aluminum chloride, will not form the black, difficultly soluble sludge-like product upon subsequent reaction with phosphorus pentasulfide. In order to obtain the results of our invention, therefore, it is necessary, first, to employ an essentially paraffinic base lubricating oil; and, second, to treat said oil with aluminum chloride.

After treatment with anhydrous aluminum chloride has progressed to the desired extent as set forth above, agitation is stopped and a sludge containing most of the aluminum chloride settles out from the main body of the oil. The sludge is drawn off and may be treated to recover aluminum chloride in accordance with methods known to the art. The supernatant body of the treated oil may contain further quantities of aluminum chloride finely dispersed therethrough, and in order to insure the removal of all aluminum chloride from the treated oil, agitation with an adsorbent clay followed by filtration may be employed. Other known methods of removing aluminum chloride from the treated oil, such as agitation with dilute sulfuric acid, may also be employed as is understood in the art. At the higher temperatures of treatment with aluminum chloride, some conversion of the paraffinic base oil to lower boiling products may take place. However, even at the highest temperature stated, namely, 300° F., such conversion is slight; but if desired, the product may be topped, that is, distilled to remove the lower boiling products overhead and to recover as a residue the bulk of the aluminum chloride treated oil having a minimum initial boiling point in the range 490° to 530° F.

The essentially paraffinic base lubricating oil treated with aluminum chloride as disclosed hereinabove is now ready for reaction with phosphorus pentasulfide. If desired, the aluminum chloride treated oil may be blended with some of the untreated charge stock without deleteriously affecting the subsequent reaction with phosphorus pentasulfide, but ordinarily not more than about 20 per cent of untreated oil should be added

to the treated product and preferably, smaller amounts should be used. However, where the color of the product is paramount, such blending may be undesirable. The reaction with phosphorus pentasulfide is accomplished by adding from 2 to 20 per cent by weight of P<sub>2</sub>S<sub>5</sub>, preferably from 5 to 10 per cent, to the aluminum chloride treated oil, or the blend disclosed above, and heating with agitation at a minimum reaction temperature of 450° F. and a maximum reaction temperature below the temperature where cracking of the oil, that is, pyrolytic decomposition of the treated oil begins. Generally, the minimum cracking temperature of the oil will vary between 490° to 530° F. depending upon the particular oil used. During the course of the reaction with P<sub>2</sub>S<sub>5</sub>, hydrogen sulfide is evolved and phosphorus and sulfur become incorporated in the aluminum chloride treated oil. When the evolution of hydrogen sulfide has nearly ceased, the temperature of the reaction mixture may be increased within the maximum temperature disclosed above, say to about 500° F. for completion of the reaction. The products so obtained are excellent improvement agents for mineral oil lubricants.

The following examples illustrate the preparation of our new improvement agent:

#### Example I

30 Three thousand gallons of a solvent-refined dewaxed paraffinic base lubricating oil were charged to a vessel equipped with an agitator and means for heating and cooling, and agitated at 275° F. while adding 4 per cent by weight of anhydrous aluminum chloride. Agitation was then continued for 4 hours. At the end of this time agitation was stopped and the bulk of the aluminum chloride settled in a sludge at the bottom of the vessel. The sludge was withdrawn, and in order to remove any remaining dispersed aluminum chloride in the body of the oil, there was added 0.2 pound per gallon of oil of an adsorbent clay, such as "Super-Filtrol," and the mixture agitated at 210° F. The mixture was then filtered and there was obtained in a yield of 84.1 per cent by volume of the original charge an aluminum chloride treated oil free of aluminum chloride and having a viscosity index of 105. To 81 parts by volume of the treated oil, there were added 19 parts by volume of the original untreated oil and, of this mixture, 8550 parts by weight were placed into a reaction vessel equipped with an agitator and means for heating and cooling. Then 450 parts by weight of P<sub>2</sub>S<sub>5</sub> were added with agitation at a temperature of 300° F. After all of the P<sub>2</sub>S<sub>5</sub> had been added, the temperature was gradually raised to 450° F. A large volume of hydrogen sulfide was evolved and when evolution of hydrogen sulfide had nearly ceased, the temperature was raised to 500° F. to complete the reaction. The reaction with P<sub>2</sub>S<sub>5</sub> from the time of its addition to the completion of the reaction took 8 hours. The reaction product was then cooled and discharged from the reaction vessel. The product had the following properties:

|                      |      |
|----------------------|------|
| Gravity, °API        | 26.1 |
| Viscosity, S.U.V.:   |      |
| 100° F.              | 651  |
| 210                  | 73.4 |
| Color, N.P.A.        | 8.0  |
| Sulfur, per cent     | 1.62 |
| Phosphorus, per cent | 1.12 |
| Neutralization No.   | 8.62 |

*Example II*

Another solvent refined dewaxed paraffinic base lubricating oil was treated with aluminum chloride under exactly the same conditions shown in Example I, except that 6 per cent by weight of aluminum chloride was used. Aluminum chloride was removed as in Example I, and the treated oil reacted with 10 per cent by weight of phosphorus pentasulfide to yield a product having the following properties:

|                         |      |
|-------------------------|------|
| Gravity, °API           | 21.7 |
| Viscosity, SUV, 100° F. | 1274 |
| Sulfur, per cent        | 1.21 |
| Phosphorus, per cent    | 2.63 |
| Neutralization No.      | 18.8 |

*Example III*

A paraffinic base oil was treated with 9 per cent by weight of aluminum chloride under conditions as given in Example I. The aluminum chloride-free reaction product was then reacted with 10 per cent by weight of phosphorus pentasulfide under the conditions shown in Example I to yield a product having the following properties:

|                         |      |
|-------------------------|------|
| Gravity, °API           | 24.9 |
| Viscosity, SUV, 100° F. | 355  |
| Sulfur, per cent        | 0.88 |
| Phosphorus, per cent    | 0.90 |
| Neutralization No.      | 0.56 |

*Example IV*

An aluminum chloride treated oil, as prepared in Example I, was treated with 10 per cent by weight of phosphorus pentasulfide at 450° F. for 6 hours to yield a product having the following properties:

|                         |      |
|-------------------------|------|
| Gravity, °API           | 23.1 |
| Viscosity, SUV, 100° F. | 1684 |
| Sulfur, per cent        | 4.41 |
| Phosphorus, per cent    | 1.69 |
| Neutralization No.      | 7.13 |

The phosphorus pentasulfide reaction products obtained in accordance with the preceding examples are excellent improvement agents for mineral oil lubricant compositions. They are readily soluble in all types of mineral oils, that is, paraffinic, naphthenic or mixed base mineral oils and, as a matter of fact, can be blended with mineral oils in proportions as high as 50 per cent by weight or higher. This excellent solubility of our new improvement agents enables the preparation of concentrated solutions of improvement agents, which may then be diluted down to the proportion desired in the final mineral oil lubricant composition. As stated, our new improvement agents confer excellent pressure-carrying, antioxidant and corrosion-

inhibiting properties on the mineral lubricating oils with which they are incorporated. For these purposes, our new improvement agents are generally added to mineral oils in minor amounts, say from 0.1 per cent to 20 per cent by weight of the mineral oil, sufficient to confer improved pressure-carrying, antioxidant and corrosion-inhibiting properties on the mineral lubricating oil compositions. When our new improvement agents are to be used for their antioxidant and corrosion-inhibiting effects, small proportions as low as 0.1 per cent by weight are sufficient to effect the improvement. When extreme pressure properties are to be conferred on a lubricating oil, higher proportions, as high as 20 per cent, may conveniently be used.

If desired, our improvement agents may be neutralized with a metallic hydroxide or an amine prior to incorporation into a mineral oil lubricant. Particularly effective improvement agents are obtained when calcium, magnesium or aluminum hydroxide are used for the neutralization. When amines are employed for the neutralization, it is preferred to employ long chain alkyl amines; but aromatic amines, aralkyl amines and cycloalkylamines, such as aniline, benzylamine and cyclohexylamine, may also be used with advantage.

The following examples illustrate the use of our new improvement agents to obtain improved mineral oil lubricant compositions:

*Example V*

A lubricating oil having excellent extreme pressure properties was prepared by blending 15 parts by weight of the improvement agent made according to Example I and 85 parts by weight of a highly refined motor oil. A comparison of the properties of the improved lubricant and the base lubricant follows:

|                                     | Unimproved Lubricant | Improved Lubricant |
|-------------------------------------|----------------------|--------------------|
| Gravity, °API                       | 29.3                 | 28.9               |
| Viscosity, SUV: 100° F.             | 246                  | 244                |
| Color, NPA                          | 1.75                 | 1.75               |
| Falex Wear Test:                    |                      |                    |
| 1000 Lbs. Gauge Load, 15 min. Wear: |                      |                    |
| No. of Teeth                        | fails                | 0                  |
| Gauge Load at Seizure: Lbs.         |                      | 1,750              |

*Example VI*

An excellent turbine oil was prepared by blending 0.3 part by weight of the improvement agent prepared in accordance with Example III and 99.7 parts by weight of a refined turbine oil base. The properties of the improved and unimproved turbine oils are as follows:

|                                                                          | Unimproved Turbine Oil | Improved Turbine Oil |
|--------------------------------------------------------------------------|------------------------|----------------------|
| Gravity: °API                                                            | 29.0                   | 28.9                 |
| Viscosity, SUV: 100° F.                                                  | 407                    | 407                  |
| 130° F.                                                                  | 192.7                  | 190.6                |
| Color, NPA                                                               | 2.75                   | 2.75                 |
| Oxidation and Bearing Corrosion Test, Method 257, Gulf:                  |                        |                      |
| Duration of Test: hr.                                                    | 48                     | 48                   |
| Oil Bath Temperature: °F.                                                | 347                    | 347                  |
| Air Rate: cc./hr.                                                        | 2,000                  | 2,000                |
| Quantity of Oil: cc.                                                     | 300                    | 300                  |
| Bearing Type                                                             |                        |                      |
| Wt. Change: Grams                                                        | Cd-Ag Cu-Pb            | Cd-Ag Cu-Pb          |
| Wt. Change: Per cent                                                     | -0.1744 -0.0188        | +0.0007 +0.0042      |
| Corrosion Test:                                                          |                        |                      |
| ASTM D 665-44 T Distilled Water, 140° F., 48 Hr. Steel Strip: Appearance | rust                   | bright               |
| Area Rusted: Per cent                                                    | 100                    | 0                    |

*Example VII*

An excellent motor oil, SAE 30 grade, was prepared by blending 1 part by weight of the improvement agent prepared in accordance with Example IV and 99 parts by weight of a highly refined paraffinic SAE 30 grade motor oil. The properties of the improved and unimproved motor oil are as follows:

|                                                         | Unimproved<br>Motor Oil | Improved<br>Motor Oil |
|---------------------------------------------------------|-------------------------|-----------------------|
| Gravity: °API                                           | 29.0                    | 29.1                  |
| Viscosity, S.U.V.: 100° F.                              | 521                     | 521                   |
| Color, N.P.A.                                           | 1.75                    | 2.0                   |
| Oxidation and Bearing Corrosion Test, Method 257, Gulf: |                         |                       |
| Duration of Test: hr.                                   | 48                      | 48                    |
| Oil Bath Temperature: °F.                               | 347                     | 347                   |
| Air Rate: cc./hr.                                       | 2,000                   | 2,000                 |
| Quantity of Oil: cc.                                    | 300                     | 300                   |
| Bearing Type                                            | Cd-Ag Cu-Pb             | Cd-Ag Cu-Pb           |
| Wt. Change: Grams                                       | -0.1744 -0.0138         | -0.054 -0.0022        |
| Wt. Change: percent                                     | -0.96 -0.08             | -0.01 -0.01           |

*Example VIII*

An SAE 20 grade motor oil was prepared by blending 1 part by weight of the additive prepared according to Example IV and 99 parts by weight of a solvent refined SAE 20 grade motor oil. The properties of the improved and unimproved motor oil are as follows:

|                                                                       | Unimproved<br>Motor Oil | Improved<br>Motor Oil |
|-----------------------------------------------------------------------|-------------------------|-----------------------|
| Gravity: °API                                                         | 29.0                    | 29.0                  |
| Viscosity, S.U.V.: 100° F.                                            | 335                     | 337                   |
| Color, N.P.A. oxidation and Bearing Corrosion Test, Method 257, Gulf: | 4.25                    | 4.25                  |
| Duration of Test: hr.                                                 | 48                      | 48                    |
| Oil Bath Temperature: °F.                                             | 347                     | 347                   |
| Air Rate: cc./hr.                                                     | 2,000                   | 2,000                 |
| Quantity of Oil: cc.                                                  | 300                     | 300                   |
| Bearing Type                                                          | Cd-Ag Cu-Pb             | Cd-Ag Cu-Pb           |
| Wt. Change: Grams                                                     | -0.2319 -0.0867         | -0.0070 -0.0112       |
| Wt. Change: percent                                                   | -1.28 -0.38             | -0.01 -0.05           |

The "Oxidation and Bearing Corrosion Test, Method 257, Gulf," referred to in the foregoing examples, is conducted as follows: An alloy bearing shell of certain commonly used standard dimensions is submerged in 300 cc. of the oil or oil composition in a 400 cc. Pyrex beaker and heated in a thermostatically controlled oil bath to 347° F. Air is then bubbled through the oil in contact with the bearing shell at the rate of 2000 cc. per hour. At the end of the 48 hours, the loss of weight and condition of the bearing shell are determined, the bearing shell being washed free of oil and dried before weighing. When determining the effectiveness of various improvement agents, the usual procedure is to run a "blank" test simultaneously with the oil composition being tested, employing for that purpose a sample of the untreated oil. In this test it is advantageous to employ commercial bearing shells. These shells comprise a suitable metal backing faced with the alloy bearing metal. In this way, the actual bearing face is subjected to severe deterioration conditions. By comparison of the results of such tests with actual service tests, we have found them to be in substantial agreement as to the suitability of particular lubricants.

As is shown in the above examples, the addition of our new improvement agents to mineral oil lubricant compositions confers excellent pressure-carrying, anti-oxidant and corrosion-inhibiting properties. At the same time, the compositions so obtained are stable in storage and use

and have a color which is substantially unaffected by the addition of the improvement agent.

While we have shown in the examples the preparation of compounded lubricating oils, our invention is not limited thereto but comprises all mineral oil lubricant compositions containing our new improvement agents, such as greases and the like.

## What we claim is:

1. The process of preparing an improvement agent for mineral oil lubricants which comprises heating a mixture consisting of an essentially paraffinic base lubricating oil and anhydrous aluminum chloride at a temperature of from 150° to 300° F., removing aluminum chloride from

30

the reaction product, and reacting said product with phosphorus pentasulfide at a temperature of from 450° F. to a maximum temperature below the minimum cracking temperature of said product to incorporate phosphorus and sulfur therein.

2. The process of preparing an improvement agent for mineral oil lubricants which comprises heating a mixture consisting of an essentially paraffinic base lubricating oil and from 1 to 20 per cent by weight of anhydrous aluminum chloride at a temperature of from 150° to 300° F., removing aluminum chloride from said product, and reacting said product with from 2 to 20 per cent by weight of phosphorus pentasulfide at a temperature of from 450° F. to a maximum temperature below the minimum cracking temperature of said product to incorporate phosphorus and sulfur therein.

3. The process of preparing an improvement agent for mineral oil lubricants which comprises heating a mixture consisting of an essentially paraffinic base lubricating oil and from 1 to 20 per cent by weight of anhydrous aluminum chloride at a temperature of from 150° to 300° F., removing aluminum chloride from the reaction product, distilling the reaction product and recovering as a residue a product having a minimum initial boiling point in the range 490° to 530° F., and reacting said product with from 5 to 10 per cent by weight of phosphorus pentasulfide at a temperature of from 450° F. to a maximum temperature below the minimum cracking

75

temperature of said product to incorporate phosphorus and sulfur therein.

4. The process of preparing an improvement agent for mineral oil lubricants which comprises heating a mixture consisting of an essentially paraffinic base lubricating oil and from 1 to 20 per cent by weight of anhydrous aluminum chloride at a temperature of from 150° F. to 300° F., removing aluminum chloride from the reaction product, reacting said product with from 5 to 10 per cent by weight of phosphorus pentasulfide at a temperature from 450° F. to a maximum temperature below the minimum cracking temperature of said product to incorporate phosphorus and sulfur therein, and dissolving the resultant 15 product in a mineral lubricating oil.

5. The product obtainable by the process of claim 1.

6. The product obtainable by the process of claim 2.

7. The product obtainable by the process of claim 3.

8. The product obtainable by the process of claim 4.

9. A lubricant composition comprising a major amount of a mineral lubricating oil base and a minor amount, sufficient to confer improved bearing corrosion-inhibiting properties on the composition, of the product obtainable by the process of claim 1.

10. A lubricant composition comprising a major amount of a mineral lubricating oil base and from 0.1 to 20 per cent by weight of the product obtainable by the process of claim 1.

11. A lubricant composition comprising a major amount of a highly refined paraffinic lubricating oil base and from 0.1 to 20 per cent of the product obtainable by the process of claim 3.

12. A turbine oil comprising a major amount of a mineral lubricating oil base and a minor amount, sufficient to confer improved bearing corrosion-inhibiting properties on the composition, of the product obtainable by the process of claim 2.

HERSCHEL G. SMITH.  
TROY L. CANTRELL.

#### REFERENCES CITED

The following references are of record in the file of this patent:

#### UNITED STATES PATENTS

| Number    | Name         | Date          |
|-----------|--------------|---------------|
| 2,242,260 | Prutton      | May 20, 1941  |
| 2,315,529 | Kelso        | Apr. 6, 1943  |
| 2,316,090 | Kelso        | Apr. 6, 1943  |
| 2,367,468 | Mixon et al. | Jan. 16, 1945 |